

W. McA. JOHNSON.  
METHOD OF CONDENSING VOLATILE METALS.  
APPLICATION FILED JAN. 8, 1908.

902,535.

Patented Oct. 27, 1908.



Fig. 2.



Witnesses:

*W. McA. Johnson*  
*C. H. Potter*

Inventor:

Woolsey McA. Johnson  
Byrnes & Townsend  
Atty's.

# UNITED STATES PATENT OFFICE.

WOOLSEY McA. JOHNSON, OF HARTFORD, CONNECTICUT.

## METHOD OF CONDENSING VOLATILE METALS.

No. 902,535.

Specification of Letters Patent. Patented Oct. 27, 1908.

Application filed January 8, 1908. Serial No. 409,861.

To all whom it may concern:

Be it known that I, WOOLSEY McA. JOHNSON, a citizen of the United States, residing at Hartford, in the county of Hartford and State of Connecticut, have invented certain new and useful Improvements in Methods of Condensing Volatile Metals, of which the following is a specification.

This invention relates broadly to the art of condensing metallic vapors, but more specifically it concerns an improved method of condensing zinc vapors whereby liquid or solid zinc may be easily obtained on a highly economical basis.

One object of this invention is to provide a commercially practicable method of rapidly condensing metallic zinc vapor in conjunction with very simple and inexpensive apparatus; which method and apparatus are of a nature permitting their operation by relatively inexperienced and unskilled workmen.

In general, this invention seeks to provide a process of the nature disclosed which, from the standpoint of commercial practice, will possess a high degree of efficiency and which will be of the greatest possible simplicity consonant with the results obtained.

Other objects and advantages will be in part obvious from the annexed drawings, and in part pointed out in the following description.

It is well known that the condensation of the metallic zinc vapor evolved from reduction furnaces has hitherto presented many difficulties in practice. Thus, should the temperature of the condensing chambers and contents be too low, a commercially satisfactory percentage of the zinc vapor will not deposit in the form of molten metal, but will in large part be deposited in the form of fume or so-called "blue powder," which requires a further treatment in order to be brought into a commercially available product. On the other hand, should the temperature be too high, the metallic zinc vapor will fail to condense with commercially economical rapidity and an undue percentage of such vapor may altogether escape condensation in the condensing chamber and may be lost or deposited as a fume in a more remote portion of the apparatus. I have, however, discovered certain conditions under which a substantially complete condensation of metallic vapors may be rapidly

effected. That is to say, my investigations have shown that by contacting the metallic vapors with a relatively large surface of molten metal having a relatively low vapor pressure, thereby the transformation of the metallic vapors into liquid form may be greatly facilitated and the flow or reaction velocity from the one condition to the other will be greatly promoted. By properly controlling the temperatures and masses, after the manner herein disclosed, the molten metal will be found to have a maximum affinity for the vaporous metal, and the condensation will proceed rapidly and may be rendered substantially complete.

By employing the molten metal in such form that it will expose a very considerable surface at low vapor pressure and by bringing the same into intimate contact with metallic vapor whose pressure is high, there will be a rapid flow from the high pressure to the low pressure (i. e., a condensation). Under these and other conditions of my process, I am enabled to properly condense an extremely large quantity of zinc vapor notwithstanding that the cubic capacity of my apparatus may be small.

In carrying out my process, I may very conveniently utilize the apparatus devised by me for that purpose and shown in the accompanying drawings, wherein:

Figure 1 is a central sectional elevation of a condenser adapted to carry out my process; and Fig. 2 is a transverse sectional elevation of the same taken in the plane of line 2—2 of Fig. 1.

The condensing chamber 1 may be constructed in suitable size and shape of any desired material, as the masonry 2, and preferably, though not necessarily, may be provided in or adjacent its lower end with a metallic collecting reservoir or basin 3 for receiving the condensed metal. The metallic vapors from the reduction furnace or other source are introduced into the condensing chamber by means of a flue 4 leading into the upper part of said chamber. The residual vapors and fixed gases are enabled to escape through the outlet 5, and for the purpose of collecting any blue powder or other valuable constituents, a prolong 6 having a discharge vent 7 for the fixed gases may be in communication with the outlet 5.

To the end that the apparatus and collecting basin may be initially heated, or main-

tained at a suitable temperature, gas burners 8 or other available form of furnace may underlie the collecting basin 3.

For the purpose of disposing the melted metal within the condensing chamber so that a relatively large superficial area may be presented to the incoming metallic vapors, I may provide one or more receptacles which preferably assume the form and function of the flues designated by 11. These flues 11 may be conveniently shaped in cross section in the form of a hollow rectangle provided with upwardly extending marginal ribs 12, or otherwise recessed or constructed to receive and retain in the form of a shallow pool or film quantities of molten metal.

A further feature of advantage which I have adopted in this apparatus resides in so arranging the flues or shelves as the case may be that the metal may overflow and shower from one flue to the other, thereby providing a different but yet efficient exposure of the molten metal to the metallic vapors. To this end, the transverse flues 11 are preferably staggered in the manner indicated so that the incoming gases may be not only brought into intimate contact with the relatively quiescent surface of the receptacles, but will also be compelled to thoroughly infiltrate through the shower of molten zinc.

In order that the metal flowing over and showering from one receptacle to another may be maintained within definite and somewhat restricted limits of temperature, I have provided flues 9 and 10 for heated gases or other fluids within or adjacent opposite sides of the condensing chamber and communicating with the transverse flues 11.

To the end that an artificial circulation of molten metal may be maintained in the condensing chamber either during the initial stages of the process or during the normal workings thereof, as the case may be, I provide means for introducing molten metal to the uppermost, and if desired to intermediary flues, and likewise, I provide means for withdrawing the molten metal from other flues or from the collecting basin. Thus, as shown on the drawings, the uppermost flue or flues 11 may be extended beyond one of the condenser walls as shown at 14 in such manner as to provide an external trough or canal communicating with the interior metal-retaining receptacles of the flues; a depending bridge wall 15 or its equivalent, serving as a seal to prevent dilution or escape of the gaseous contents of the condensing member. A like construction may be given the collecting basin as shown at 16. These extensions of the flues and of the collecting basin are for the purpose of permitting the molten metal from the collecting basin, or from any other part of apparatus, to be returned to the upper level of the condenser, thereby providing any desired rate of flow or mass of metal

within the condenser in the liquid state. The transfer of the metal from the basin 3 to the trough 14 may be effected or accomplished by any desired means, as by means of a ladle 17, by any suitable type of mechanical conveyor, by a rotary pump working at high temperatures, or equivalent constructions.

My process may be carried out as follows: The vapors may be derived as usual from a suitable reduction or volatilizing furnace, which, however, in this case may be of a relatively large capacity. These vapors enter the condenser through the flue 4 and flow downwardly therethrough. When employed for condensing vapors of metallic zinc, which will enter the chamber at a temperature of approximately 1100° C., the gases passing through the flues 9 and 11 will preferably be given a temperature range of from 450° C. to 700° C. This will ordinarily suffice to maintain the molten metal within the condensing chamber at a proper temperature relative to that of the zinc vapor to be condensed. At the start of the process the condenser will preferably be provided with suitable quantity of molten metal by extraneously introducing the same upon the upper range of flues 11 and permitting it to shower from flue to flue filling the receptacles of all the flues. At this stage, the metal within the collecting basin 3 may be maintained in a molten state and at a proper temperature by the application of heat from the burner 8. It will be understood that a mechanical or artificial circulation may be thus maintained and that such circulation may be greatly augmented and at times supplanted by the condensation of considerable amounts of the metallic vapor. That is to say, under proper conditions of normal working, the metallic vapors may condense so rapidly and in such quantities as to maintain the drip flow or shower of molten metal from flue to flue, thereby automatically providing relatively large surfaces of molten metal at proper temperatures within the condensing chamber and in intimate contact with the vapors to be condensed. Should, however, the condensation be not sufficiently rapid for this purpose, or in case uncondensed metallic vapors should be found to escape from the condenser, it will be desirable to mechanically increase the circulation in the manner above indicated.

As many changes could be made in the above construction and many apparently widely different embodiments of this invention could be made without departing from the scope thereof, it is intended that all matter contained in the above description or shown in the accompanying drawings shall be interpreted as illustrative and not in a limiting sense.

I claim:

1. The method of condensing volatile

- metals which consists in bringing metallic vapors into contact with a body of molten metal, and controlling the conditions to secure substantially complete condensation of 5 said vapors.
2. The method of condensing volatile metals which consists in bringing metallic vapors into contact with a body of molten metal, and regulating the mass of the molten metal in contact with the vapors to secure 10 substantially complete condensation of said vapors.
3. The method of condensing volatile metals which consists in bringing metallic vapors into contact with a body of molten metal, and regulating the temperature and mass of the molten metal in contact with the vapors to secure substantially complete condensation of said vapors. 15
4. The method of condensing metallic vapors which consists in exposing said vapors to a relatively large surface of a circulating molten metal. 20
5. The method of condensing metallic vapors which consists in exposing said vapors to a relatively large surface of a circulating molten metal and maintaining said metal at a temperature such that its vapor pressure is materially less than that of said metallic 25 vapor.
6. The method of condensing metallic vapors consisting in exposing a metallic vapor to a shower of molten metal.
7. The method of condensing metallic vapors which consists in simultaneously exposing said vapors to a relatively large horizontal surface of a circulating molten metal and to a shower of said metal. 30
8. The method of condensing metallic vapors which consists in simultaneously exposing said vapors to a relatively quiescent surface and to a shower of a molten metal, and withdrawing the excess of molten metal formed by the condensation of said vapors. 35
9. The method of condensing metallic vapors consisting in exposing a metallic vapor to a plurality of relatively quiescent surfaces of a circulating molten metal and simultaneously exposing said vapor to a shower of molten metal. 40
10. The method of condensing volatile metals which consists in establishing a flow of molten metal between condensing surfaces, and condensing vapors of the same metal by contact with the molten metal. 45
11. The method of condensing volatile
- metals which consists in repeatedly circulating a body of molten metal between condensing surfaces, and condensing vapors of the same metal by contact with the molten metal. 50
12. The method of condensing volatile metals which consists in providing a plurality of independent bodies of molten metal within a condensing chamber, maintaining a flow of metal between said bodies and condensing vapors of the same metal by contact with the molten metal. 55
13. The method of condensing volatile metals which consists in providing a plurality of independent bodies of molten metal within a condensing chamber, maintaining a flow of metal between said bodies in the form of a freely-falling stream, and condensing vapors of the same metal by contact with the molten metal. 60
14. The method of condensing zinc vapors which consists in establishing a flow of molten zinc between condensing surfaces, and condensing zinc vapors by contact with the molten metal. 65
15. The method of condensing zinc which consists in repeatedly circulating a body of molten zinc between condensing surfaces, and condensing zinc vapors by contact with the molten metal. 70
16. The method of condensing zinc which consists in providing a plurality of independent bodies of molten zinc within a condensing chamber, maintaining a flow of zinc between said bodies, and condensing zinc vapors by contact with the molten metal. 75
17. The method of condensing zinc which consists in providing a plurality of independent bodies of molten zinc within a condensing chamber, maintaining a flow of zinc between said bodies in the form of a freely-falling stream, and condensing zinc vapors by contact with the molten metal. 80
18. The method of condensing volatilized metals which consists in conducting metallic vapors into presence of a body of the same metal in a molten state, and regulating the exposed surface of molten metal to secure a substantially complete condensation of the vapors. 85
- In testimony whereof, I affix my signature in presence of two witnesses.
- WOOLSEY MCA. JOHNSON.
- Witnesses:
- CHAS. H. BRISCOE,  
GEO. B. THAYER.